# EUROPEAN PATENT SPECIFICATION

(11) **EP 3 243 930 B1**
(45) Date of publication and mention of the grant of the patent: **14.10.2020**
(21) Application number: 17170140.2
(22) Date of filing: 09.05.2017
(51) Int. Cl.: C23C 30/00, B05B 17/06, B05D 1/02

(54) **PROCESS FOR APPLYING ANTI-GALLANT COATING WITHOUT MASKING**
VERFAHREN ZUM AUFBRINGEN EINER ANTI-FRESSBESCHICHTUNG OHNE MASKIERUNG
PROCÉDÉ D'APPLICATION DE REVÊTEMENT ANTI-GALLANT SANS MASQUAGE

(30) Priority: 09.05.2016 US 201615150084
(43) Date of publication of application: 15.11.2017
(73) Proprietor: United Technologies Corporation, Farmington, CT 06032 (US)
(72) Inventor: BARRON, Alan C., Jupiter, FL Florida 33458 (US)
(74) Representative: Dehns

(56) References cited:
- JP-A- H0 721 553
- US-A1- 2005 098 101
- US-A1- 2007 031 611
- US-A1- 2012 183 799

## Description

### BACKGROUND

When metals are attached to each other, a form of wear called galling can occur between the surfaces where they are connected or adhered. When metals gall, the material is pulled with the contacting surface over time. This is caused by a combination of friction and adhesion between the surfaces, followed by a tearing of crystal structure. This can leave some materials friction welded to adjacent surfaces. Metals in particular gall due to their atomic structures. Galling can occur on metal surfaces where there is a lack of lubrication between the surfaces.

In many industries, including aerospace, medical devices, oil and gas, and fasteners, galling is prevented by the used of anti-gallant coatings. Anti-gallant coatings are chemical coatings applied to the surface of metals which are connected and prevent later galling. Anti-gallant coatings can have a variety of chemical compositions and are used to protect specific metal parts from galling. The anti-gallant coating chemically reacts with adjacent metal parts when stress is applied to the adhesion.

The application of anti-gallant coatings has previously been accomplished by mechanical means such as brushes, sponges and rollers, in addition to air sprays. These methods are cumbersome both because they are imprecise and may result in poor quality coatings which adhere to other parts of the item, not just the metal parts of interest. Mechanical methods that require a human hand to apply the coating, such as brushes or sponges, may miss parts, apply the coating unevenly, or get the coating on unwanted areas. Traditional air sprays are also imprecise, as a large amount of the coating ends up in the atmosphere as opposed to on the surface of interest. Additionally, overspray resulting from air sprays or similar methods creates uneven coatings, leaving a signature and feathering on the edges of the coated part.

Industry methods have long used masking to prevent other parts from being touched or coated during the anti-gallant coating method. Masking is a time-consuming preparation process in which parts of the device are covered or "masked" to prevent the application of anti-gallant coating to that part. This process greatly increases the time and money spent to apply anti-gallant coatings to certain metal parts. If masking is done improperly, there is additional cost of poor quality when the device must be cleaned and the anti-gallant coating re-applied to the correct areas, if the device can be used after improper masking.

Today, industry standards for applying anti-gallant coatings use mechanical methods which can cause inconsistencies, thick coatings, imprecise applications, feathering on edges, and require masking of nearby metal parts when the substrate is being coated.

US 2007/031611 A1 discloses a prior art ultrasound medical stent coating method and device.

US 2005/098101 A1 discloses a prior art apparatus for manufacturing a fuel cell membrane electrode assembly.

US 2012/183799 A1 discloses prior art sinter bonded porous metallic coatings.

JP H07 21553 A discloses a prior art device for producing a lubricative layer of magnetic recording medium.

### SUMMARY

From a first aspect, the invention provides a method for applying anti-gallant coating to parts, as recited in claim 1.

The invention also provides a system for applying anti-gallant coating to parts, as recited in claim 5.

Features of embodiments of the invention are set forth in the dependent claims.

### BRIEF DESCRIPTION OF THE DRAWINGS

FIG. 1 is a perspective view of an ultrasonic sprayer attached to a robotic arm spraying a metal sheet with anti-gallant coating.
FIG. 2 is a flow chart of a method of applying an anti-gallant coating to a part without masking.

### DETAILED DESCRIPTION

Leveraging ultrasonic nozzle technology and high precision machines, such as robotic arms, to apply anti-gallant coatings to substrates allows not only for higher precision in coatings, but also for evenly, consistently applied coatings without feathering that will wear at the same rate, less environmental harm due to minimal coating release into the atmosphere, and the elimination of the need of masking, resulting in lower costs and time.

Previous methods have not used high precision instruments, such as ultra-sonic nozzles, or robotic arms, to apply anti-gallant coatings. High precision ultra-sonic nozzles, such as those disclosed in U.S Patent No. 9,242,049, offer a coating spray which is much more precise than traditional paint spray nozzles. Unlike traditional spray nozzle systems, ultrasonic spray nozzle systems are more environmentally friendly due to their higher precision and resulting lower waster.

Similarly, anti-gallant coating methods have not leveraged technology such as precision devices or robotic arms. Precision devices such as gantry, six-axis or selective-compliance-articulated robotic arms, cam-operated articulable arms, or computer numerical control machines, are many times more precise than the human hand, and allow for repeatable, consistent coatings.

**FIG. 1** is a schematic diagram of system 10 for applying anti-gallant coating. System 10 includes robotic arm 12, container 14, ultrasonic nozzle 16, substrates 18, 20, controller 22 and user interface 24.

Robotic arm 12 is an example of a high precision device used to apply precise, even coatings. In Figure 1, robotic arm 12 is a gantry robot which had three prismatic joints and whose axes coincide with Cartesian coordinates. Robotic arm 12 can be programmed through user interface 24, and both movement of the arm and release of spray can be controlled through programming. Robotic arm 12 can be a gantry, a six-axis or a selective-compliance-articulated robot arm (SCARA). A gantry arm, also known as a Cartesian arm, is a mechatronic device which uses motors and linear actuators to position a tool, such as an ultrasonic nozzle. A gantry arm makes movements along X, Y and Z coordinates. A SCARA arm similarly moves along X, Y, and Z axes but may also incorporate a θ axis. Six-axis arms offer more directional control and are similar to the human arm in movement style, but with higher precision. All three types offer accuracy ranges if at least 0.1 mm, while varying versions of gantry arms can be as precise as 10 µm. Alternatively, the precision device could be any type of robotic device useable for spray coating application, such cam-operated articulable arms or a computer numerical control (CNC) machine, which are simpler and may be programmed with a repeatable set of movements.

Container 14 holds an anti-gallant coating material. Anti-gallant coatings are used particularly with stainless steel and other corrosion-resistant metal alloys which are prone to galling. Galling is a severe form of adhesive wear which occurs due to the transfer of material between sliding surfaces. Metallic surfaces are prone to galling particularly when there is poor lubrication. This occurs in a variety of industries and metal parts, including engine bearings, hydraulic cylinders, gas turbine vanes and blades, valves, screw threads, pistons and actuators. Anti-galling coatings can include hard anodized coatings, silver plated coatings, thermal spray coatings, electroless nickel coatings, dry lubrications, and many other industry-specific coatings.

Ultrasonic nozzle 16 is attached to robotic arm 12. Ultrasonic nozzles allow for the application of precise, thin film coatings without feathering effects. While traditional mechanical methods such as rollers or brushes create thick or uneven coatings, traditional pressure nozzle spray applications are imprecise and leave up to ninety percent of the coating material dispersing in the air around the substrate instead of sticking to the substrate. Ultrasonic nozzle sprayers, in contrast, produce a fine mist spray which is focused. Ultrasonic nozzles atomize liquids using high frequency sound waves, which are outside of the human hearing range, rather than forcing liquid through a small orifice as in traditional pressure spray nozzles. Ultrasonic nozzles result in a more uniform dispersion of coating particles in very thin layer due to the suspension of the particles in the nozzle throughout spraying. Commercially available ultrasonic nozzles allow for adjustment of the spray pattern within 1.78 mm to 25 mm, depending on the specific nozzle. This reduces over-spraying, which both reduces atmosphere contamination and prevents a feathering effect on the edges of the sprayed part, allowing for an evenly distributed coating without any signature.

Substrate 18 is an example of a metal part which is to be coated with anti-gallant coating. Many metals, including aluminum and stainless steel, can gall easily, while others, such as steel or brass, are less prone to galling. Substrate 20 is an example of a metal part which is attached to substrate 18, but should not be coated with anti-gallant coating. In prior art, substrate 20 would be masked to prevent application of the anti-gallant coating to that part. Masking is a method of protecting certain parts of an item from exposure to the coating. With masking, certain parts are painstakingly covered or sealed off to ensure no coating comes into contact with those parts. Incorrect masking can lead to further problems and repeated attempts to apply anti-gallant coatings. However, with the use of a high-precision system for applying the coating, substrate 20 does not need to masked, saving time, money, and potential errors.

Controller 22 is used to control the movement of the robotic arm and the spray of the ultrasonic nozzle. Controller 22 may be either programmable through user interface 24, or controlled directly by the user to create a path for robotic arm 12 to follow. Specifically, controller 22 is complex enough to allow coating of substrate 18 but not coating of substrate 20. User interface 24 allows programming and control of robotic arm 12. Once programmed, controller 22 includes memory that stores instructions and data (programming) that allows robotic arm 12 to be moved precisely along a defined path to replicate application of the anti-gallant coating on multiple parts.

System 10 can be used to apply anti-gallant coatings of varying thickness to small, specific areas of substrates without masking.

**FIG. 2** is a flow chart of method 28 for applying an anti-gallant coating to a metal part without masking. Method 28 includes loading instructions (step 30), loading container (step 32), securing sprayer (step 34), mounting metal parts (step 36), spraying metal parts on area of interest (step 38), and removing metal parts (step 40).

Method 28 begins with step 30, when the user programs a precise manipulation device. As discussed earlier, the precise manipulation device may be a robotic arm, such as arm 12 pictured in Figure 1, any other type of camera operated articulable arm, or a CNC device. Depending on the requirements for the particular type of device, the programming step may include programming a simple, repeatable set of movement and spraying, or it may be complex.

Next, in step 32, the user loads the anti-gallant coating material into the ultrasonic sprayer, such as sprayer 16 pictured in Figure 1. Here, the user can select one of many types of anti-gallant coatings materials, depending on the substrate being coated. This can include dry lubrications, and many other industry-specific coatings, which work differently with varying substrates.

In step 34, the user secures the ultrasonic sprayer to the precise manipulation device. The ultrasonic sprayer must be secure such that the movement of the precise manipulation device will not shake the ultrasonic sprayer, altering the spray pattern. The ultrasonic sprayer can be secured through fasteners, clasps, or any other reasonable method for attachment to the manipulation device.

Next, in step 36 the items to be coated are placed in range of the precise manipulation device. In Figure 1, the example given is substrate 18. Once the substrate is secured, there is no need to mask unwanted parts. Instead, the precise manipulation device can be programmed specifically, with more precision than a human hand, to spray only parts that should be coated with the anti-gallant coating. Even without masking, the high precision of the ultrasonic sprayer and precise manipulation device prevent feathering on the edges of the substrate.

In step 38, the program for the precise manipulation device should be run, carefully controlling both spray and movement. This process can be completed in a "quiet" environment, as the ultrasonic sprayer does not produce waste associated with traditional pressure sprayers and there is no need to keep a fan or vacuum to eliminate that waste. The coating that is applied to the part will be thin, even, and will not contain a signature such as feathering. Finally, once coating is completed, the substrates or other coated items should be removed from their stationary position (step 40).

The present invention can produce a coating that is uniform in thickness, which is defined as thickness with less than twenty percent variation. Additionally, there is substantially no feathering along the edges of the coating, or any other signature left by the coating method, that can occur when other methods are utilized.

Method 28 presents unique benefits in the anti-gallant coating process that have not previously been addressed. First, the method presented does not require masking. Currently, masking in anti-gallant coating processes is more time, energy and money consuming than applying the anti-gallant coating itself. The use of the ultrasonic spray system eliminates the need for masking because of its high accuracy and precision. Additionally, the use of a robotic arm or other manipulation device allows for higher precision and repeatability than using a human hand to apply the coating. Moreover, the coating that is applied to the substrate is uniform in thickness, and can be applied very thinly to materials on which a thick coating is not desired. Finally, the use of a quiet environment in which there is no aerosol waste is an environmental improvement.

Therefore, it is intended that the invention not be limited to the particular embodiment(s) disclosed, but that the invention will include all embodiments falling within the scope of the appended claims.

## Claims

1. A method for applying anti-gallant coating to a part, the method comprising:
positioning a part to receive anti-gallant material dispensed by an ultrasonic sprayer (16) attached to a precise manipulation device (12); and
moving the ultrasonic sprayer (16) with the precise manipulation device (12) according to a spray path with a positional accuracy within a range of 10 µm to 0.1 mm; and
spraying the anti-gallant material out of the ultrasonic sprayer (16) while moving the ultrasonic sprayer (16) to form an anti-gallant coating on a portion of the part defined by the spray path.

2. The method of claim 1, and further comprising:
loading instructions in a controller (22), wherein the instructions specify movement of the precise manipulation device (12) and spraying of the ultrasonic sprayer (16), and wherein the instructions define the spray path; and
executing the instructions in the controller (22) to control movement of the precise manipulation device (12) and operation of the ultrasonic sprayer (16) to spray anti-gallant material onto a defined area or areas of the part.

3. The method of claim 2, wherein the controller controls the precise manipulation device (12) and the ultrasonic sprayer (16) to produce a coating with substantially no feathering.

4. The method of claim 1, and further comprising spraying the anti-gallant material onto the part in an environment without a fan or vacuum.

5. A system (10) for applying anti-gallant coating to a part, the system comprising:
a container (14) for holding a supply of anti-gallant material;
an ultrasonic nozzle (16) connected to the container (14) that dispenses the anti-gallant material; and
a precise manipulation device (12) that moves the ultrasonic nozzle (16) with respect to a part along a spray path with a positional accuracy within a range of 10 µm to 0.1 mm to deposit an anti-gallant coating on a defined area or areas of the part.

6. The system of claim 5, further comprising a controller (22) containing a memory configured to store and deliver instructions, wherein the instructions specify movement of the precise manipulation device (12) and spraying of anti-gallant material by the ultrasonic nozzle (16).

7. The system of claim 6, wherein the controller (22) controls the precise manipulation device (12) and the ultrasonic nozzle (16) to produce the anti-gallant coating with substantially no feathering.

8. The system of any of claims 5 to 7, wherein the ultrasonic nozzle (16) is configured to spray anti-gallant material onto the part in an environment without a fan or vacuum.

9. The method or system of any preceding claim, wherein the precise manipulation device (12) comprises at least one of a robotic arm (12) or a computer numerical control.

10. The method or system of any preceding claim, wherein the ultrasonic nozzle (16) is configured to adjust spray of the anti-gallant material within a spray width of 1.78 mm to 25 mm.

## Patentansprüche

1. Verfahren zum Aufbringen einer Anti-Fressbeschichtung an einem Teil, wobei das Verfahren Folgendes umfasst:
Positionieren eines Teils, um ein Anti-Fressmaterial zu empfangen, das von einem Ultraschallzerstäuber (16) abgegeben wird, der an einer präzisen Manipulationsvorrichtung (12) angebracht ist; und
Bewegen des Ultraschallzerstäubers (16) mittels der präzisen Manipulationsvorrichtung (12) gemäß einer Sprühbahn mit einer Positionsgenauigkeit innerhalb eines Bereichs von 10 µm bis 0,1 mm; und
Sprühen des Anti-Fressmaterials aus dem Ultraschallzerstäuber (16) während eines Bewegens des Ultraschallzerstäubers (16), um eine Anti-Fressbeschichtung an einem Abschnitt des Teils zu bilden, der durch die Sprühbahn definiert wird.

2. Verfahren nach Anspruch 1, ferner Folgendes umfassend:
Laden von Anweisungen in eine Steuerung (22), wobei die Anweisungen eine Bewegung der präzisen Manipulationsvorrichtung (12) und ein Sprühen des Ultraschallzerstäubers (16) spezifizieren und wobei die Anweisungen die Sprühbahn definieren; und
Ausführen der Anweisungen in der Steuerung (22), um eine Bewegung der präzisen Manipulationsvorrichtung (12) und einen Betrieb des Ultraschallzerstäubers (16) zu steuern, um Anti-Fressmaterial auf einen definierten Bereich oder definierte Bereiche des Teils zu sprühen.

3. Verfahren nach Anspruch 2, wobei die Steuerung die präzise Manipulationsvorrichtung (12) und den Ultraschallzerstäuber (16) steuert, um eine Beschichtung herzustellen, die im Wesentlichen keine weichen Kanten aufweist.

4. Verfahren nach Anspruch 1, ferner ein Sprühen des Anti-Fressmaterials auf das Teil in einer Umgebung ohne Gebläse oder Vakuum umfassend.

5. System (10) zum Aufbringen einer Anti-Fressbeschichtung auf einem Teil, wobei das System Folgendes umfasst:
einen Behälter (14) zum Halten eines Vorrats an Anti-Fressmaterial;
eine Ultraschalldüse (16), die mit dem Behälter (14) verbunden ist, der das Anti-Fressmaterial abgibt; und
eine präzise Manipulationsvorrichtung (12), die die Ultraschalldüse (16) in Bezug auf ein Teil mit einer Positionierungsgenauigkeit innerhalb eines Bereichs von 10 µm bis 0,1 mm entlang einer Sprühbahn bewegt, um eine Anti-Fressbeschichtung auf einem definierten Bereich oder definierten Bereichen des Teils abzulagern.

6. System nach Anspruch 5, ferner eine Steuerung (22) umfassend, die einen Speicher enthält, der dazu konfiguriert ist, Anweisungen zu speichern und auszugeben, wobei die Anweisungen eine Bewegung der präzisen Manipulationsvorrichtung (12) und ein Sprühen von Anti-Fressmaterial durch die Ultraschalldüse (16) spezifizieren.

7. System nach Anspruch 6, wobei die Steuerung (22) die präzise Manipulationsvorrichtung (12) und die Ultraschalldüse (16) steuert, um die Anti-Fressbeschichtung herzustellen, die im Wesentlichen keine weichen Kanten aufweist.

8. System nach einem der Ansprüche 5 bis 7, wobei die Ultraschalldüse (16) dazu konfiguriert ist, Anti-Fressmaterial in einer Umgebung ohne Gebläse oder Vakuum auf das Teil zu sprühen.

9. Verfahren oder System nach einem der vorhergehenden Ansprüche, wobei die präzise Manipulationsvorrichtung (12) mindestens eines von einem Roboterarm (12) oder einer CNC-Steuerung (Computer Numerical Control) umfasst.

10. Verfahren oder System nach einem der vorhergehenden Ansprüche, wobei die Ultraschalldüse (16) dazu konfiguriert ist, ein Sprühen des Anti-Fressmaterials innerhalb einer Sprühbreite von 1,78 mm bis 25 mm anzupassen.

## Revendications

1. Procédé d'application de revêtement anti-galant sur une pièce, le procédé comprenant :
le positionnement d'une pièce pour recevoir un matériau anti-galant distribué par un pulvérisateur à ultrasons (16) fixé à un dispositif de manipulation précise (12) ; et
le déplacement du pulvérisateur à ultrasons (16) avec le dispositif de manipulation précise (12) selon un trajet de pulvérisation avec une précision de positionnement comprise dans une plage allant de 10 µm à 0,1 mm ; et
la pulvérisation du matériau anti-galant hors du pulvérisateur à ultrasons (16) tout en déplaçant le pulvérisateur à ultrasons (16) pour former un revêtement anti-galant sur une partie de la pièce définie par le trajet de pulvérisation.

2. Procédé selon la revendication 1, et comprenant en outre :
le chargement d'instructions dans un dispositif de commande (22), dans lequel les instructions spécifient le déplacement du dispositif de manipulation précise (12) et la pulvérisation du pulvérisateur à ultrasons (16), et dans lequel les instructions définissent le trajet de pulvérisation ; et
l'exécution des instructions dans le dispositif de commande (22) pour commander le mouvement du dispositif de manipulation précise (12) et le fonctionnement du pulvérisateur à ultrasons (16) pour pulvériser un matériau anti-galant sur une zone ou des zones définies de la pièce.

3. Procédé selon la revendication 2, dans lequel le dispositif de commande commande le dispositif de manipulation précise (12) et le pulvérisateur à ultrasons (16) pour produire un revêtement sans pratiquement aucun adoucissement.

4. Procédé selon la revendication 1, et comprenant en outre la pulvérisation du matériau anti-galant sur la pièce dans un environnement sans ventilateur ni vide.

5. Système (10) d'application d'un revêtement anti-galant sur une pièce, le système comprenant :
un récipient (14) pour contenir une réserve de matériau anti-galant ;
une buse à ultrasons (16) reliée au récipient (14) qui distribue le matériau anti-galant ; et
un dispositif de manipulation précise (12) qui déplace la buse à ultrasons (16) par rapport à une pièce le long d'un trajet de pulvérisation avec une précision de positionnement dans une plage allant de 10 µm à 0,1 mm pour déposer un revêtement anti-galant sur une zone ou des zones définies de la pièce.

6. Système selon la revendication 5, comprenant en outre un dispositif de commande (22) contenant une mémoire configurée pour stocker et délivrer des instructions, dans lequel les instructions spécifient le mouvement du dispositif de manipulation précise (12) et la pulvérisation de matériau anti-galant par la buse à ultrasons (16).

7. Système selon la revendication 6, dans lequel le dispositif de commande (22) commande le dispositif de manipulation précise (12) et la buse à ultrasons (16) pour produire le revêtement anti-galant sans pratiquement aucun adoucissement.

8. Système selon l'une quelconque des revendications 5 à 7, dans lequel la buse à ultrasons (16) est configurée pour pulvériser un matériau anti-galant sur la pièce dans un environnement sans ventilateur ni vide.

9. Procédé ou système selon une quelconque revendication précédente, dans lequel le dispositif de manipulation précise (12) comprend au moins l'un d'un bras robotique (12) ou d'une commande numérique informatique.

10. Procédé ou système selon une quelconque revendication précédente, dans lequel la buse à ultrasons (16) est configurée pour régler la pulvérisation du matériau anti-galant dans une largeur de pulvérisation de 1,78 mm à 25 mm.
